

Patented Mar. 24, 1925.

## UNITED STATES PATENT OFFICE.

WILHELM HELMUT SCHWEITZER, OF HEIDELBERG, GERMANY, ASSIGNOR, BY MESNE ASSIGNMENTS, TO AMERICAN LANIL CORPORATION, A CORPORATION OF NEW JERSEY.

## PROCESS FOR OBTAINING NEW EFFECTS ON ANIMAL FIBERS.

No Drawing.

Application filed November 17, 1922. Serial No. 601,647.

To all whom it may concern:

Be it known that I, WILHELM HELMUT SCHWEITZER, a citizen of the Republic of Germany, and resident of Heidelberg, Baden, Germany, have invented a new and useful Process for Obtaining New Effects on Animal Fibers, of which the following is a full, clear, and exact specification.

It is known to treat animal fibers with paraffine, wax and the like, whereby this treatment is commonly combined with the use of an alkaline bath. Now, I have found that new, particularly beautiful, bright color effects can be obtained on chlorinated or otherwise oxidized wool if the subsequent treatment with paraffine or other wax is performed on the chlorinated or otherwise oxidized wool by way of direct application thereof, that is without any intermediate alkaline treatment. Wool thus treated shows, when being in use to cover body parts, the surprising property of keeping them warm, probably by reason of a reduction of the heat conductibility of the fibers, whereby the preliminary chlorination or other oxidation of the fibers renders them particularly proper for this paraffine or other wax impregnation. The treatment of the chlorinated or otherwise oxidized wool with

paraffine or other wax may be effected before or after the dyeing or without any dyeing operation.

Example: 100 kilos of knitting yarn of wool are chlorinated and dyed in any known manner. After being dried, the material is passed through a bath of molten paraffine, then squeezed out and liberated by known means from any excess of paraffine. By reason of the chlorination of the fibers, the same become extremely able to absorb the impregnating paraffine mass, so that a thorough impregnation of the fibers is obtained and kept up even on repeated washing.

What I claim is:

The process of treating animal fibers which consists in subjecting chlorinated or oxidized wool to a bath of wax by direct application without intermediate alkaline treatment, and then removing any excess of wax.

In witness whereof I have hereunto signed my name this 2nd day of November, 1922, in the presence of two subscribing witnesses.

WILHELM HELMUT SCHWEITZER.

Witnesses:

AMAND BAUN,  
JULIA A. DURST.